

March 5, 1957

KIYOTO MATSUZUKA

2,784,074

METHOD OF TREATING IRON ORES CONTAINING CHROMIUM

Filed Nov. 5, 1953

3 Sheets-Sheet 1

FIG.1.



INVENTOR.

BY KIYOTO MATSUZUKA

Underoth, Lind & Brack  
Attorneys

March 5, 1957

KIYOTO MATSUZUKA

2,784,074

METHOD OF TREATING IRON ORES CONTAINING CHROMIUM

Filed Nov. 5, 1953

3 Sheets-Sheet 2

FIG.2. Extraction Percentages of Cr, Al, Na & SiO<sub>2</sub> (For Na<sub>2</sub>CO<sub>3</sub> = 15% and various weights of Ca(OH)<sub>2</sub>)



FIG.3. Constitution of pellets (For Na<sub>2</sub>CO<sub>3</sub> = 15% and various weights of Ca(OH)<sub>2</sub>)



INVENTOR.

KIYOTO MATSUZUKA  
BY

Studer & Lavel & Roseck  
Attorneys

March 5, 1957

KIYOTO MATSUZUKA

2,784,074

METHOD OF TREATING IRON ORES CONTAINING CHROMIUM

Filed Nov. 5, 1953

3 Sheets-Sheet 3

FIG. 4. Extraction Percentages of Cr & Al  
(For  $\text{Na}_2\text{CO}_3$ —12.5%, 15%, 20% & 25%)



FIG. 5. Weights of Cr in Pellets (For  $\text{Na}_2\text{CO}_3$ —12.5%, 15%, 20% & 25%)



INVENTOR.

KIYOTO MATSUZUKA  
BY

Stenderup, Lied & Prell  
Attorneys

1

2,784,074

## METHOD OF TREATING IRON ORES CONTAINING CHROMIUM

Kiyoto Matsuzaka, Kumamoto-ken, Japan, assignor to  
Yawata Iron & Steel Co., Ltd., Tokyo, Japan

Application November 5, 1953, Serial No. 390,376

Claims priority, application Japan February 14, 1953

9 Claims. (Cl. 75—3)

This invention relates to a method of removing chromium from iron ores containing chromium and particularly to a method of recovering chromium from lateritic ore and of making said ores especially suitable as raw materials for producing iron.

Laterite is representative of iron ores containing chromium and it is as such representative that it is dealt with in the following. Laterite as known is an air-slaked product of serpentine and the amount of its deposits is said to be inexhaustible. It is produced in quantities in every country of the world. Laterite, for example, produced in the Philippines contains 47.7 to 51.4% Fe, 2.10 to 2.74% Cr, 4.50 to 7.52%  $Al_2O_3$ , 1.90 to 3.33%  $SiO_2$  and small amounts of Ni, Co and Mn. The main constituent of this ore is ferric oxide. The result of analysis by heat shows that this ore has 5.5% water of crystallization at 200 to 250° C. It can be presumed from the amount of dehydration that all  $Fe_2O_3$  exists in the form of  $Fe_2O_3 \cdot H_2O$  (needle iron ore). Needless to say, it is judged from the constitution of said ore that some gelled iron oxide containing water and  $Fe_2O_3 \cdot 3H_2O$  also exist. Alumina seems to exist as  $Al_2O_3 \cdot 3H_2O$  or  $Al_2O_3 \cdot H_2O$ . Silicic acid exists as silica, gelled silicic acid and silicate. Chromium exists mostly as chromite ( $FeO \cdot Cr_2O_3$ ) and partly as chromate. The chromite is so brittle in nature that it can be easily crushed by finger tips. Its grains are so fine as to be muddy. The fine grains of limonite are adsorbed by chromite or envelop chromite; this state continues the same all through to the fine grains of chromite. When both of these minerals are crushed for physical separation, chromite will be readily finely ground, will become colloidal and will be very difficult to separate by gravity or any other method. This is the main cause of the difficulty of dressing this ore. As regards the matter of removing chromium for the sake of utilizing laterite, various methods have been tested and reported in the United States on ores produced in Cuba, and in Japan on ores produced in the Philippines and Japan proper. These respective methods and the results of laboratory tests are discussed in the following.

### (1) DRESSING BY GRAVITY

This is to utilize the difference of specific gravity between iron ore and chromite. In U. S. Patent No. 2,363,315 aiming at separating nickel and chromium from Cuban laterite, Mr. John D. Grothe purports to achieve separation by utilizing the difference of specific gravity between magnetite (5.1 specific gravity) produced by reduction and roasting and chromite (4.4 specific gravity); in the case of removing chromium, this method being especially named flotation. However, it is found in the light of the theory in dressing that such fine grains cannot be well separated by the specific gravity difference of 0.7. As the assignee of patentee, Dorr Company, confesses, this method can hardly be reliably industrialized.

2

### (2) DISPERSION

When laterite is thrown into water and stirred, it will readily collapse and will sink down after a while. However, if a small amount of a dispersing agent such as for example, alkali is added thereto and the mixture is stirred and left alone, the fine grains of limonite will be dispersed and floated. The deposit contains comparatively much chromium. It is intended to attain the object of dressing by separating the floating substance and the deposit by an adequate method. The results of tests made by using 20% NaOH as a dispersing agent on an Omonhon specimen (containing 2.74% chromium) are now listed in the following:

| No. | Raw Material in g. | Water in l. | Dispersing Agent 20% NaOH in cc. | Dispersed Weight in Percent | Substance Chromium in Percent |
|-----|--------------------|-------------|----------------------------------|-----------------------------|-------------------------------|
| 20  | 1. 300             | 4           | .5                               | 45                          | 1.86                          |
|     | 2. 300             | 4           | 10                               | 47                          | 1.75                          |
|     | 3. 300             | 4           | 20                               | 49                          | 1.87                          |
|     | 4. 300             | 6           | 20                               | 46                          | 1.33                          |

As seen from the above results of experiments, in this method, the percentage of the removal of chromium is low (below 50%) and the percentage of collection of iron ores is below 50%, being out of the question.

This method was named emulsion dressing by the Heavy Metal Research Laboratory established in Japan during World War II. It is found in the light of the reports of experiments made by this method on various kinds of laterite produced in various producing places as published in Reports of the Heavy Metal Research Institute, 1st edition, December 1944, that, though some favorable results have been shown in some producing places, the percentage of the removal of chromium and the percentage of collection of iron ores are not favorable and the drying operation after separation is difficult. In view of such results, this method is never suited to treatment of large quantities.

### (3) ADDITION OF SODA ASH

This is like the method of the present invention to be described later and is a method wherein chromium is extracted as sodium chromate by merely adding soda ash to the raw material and heating the mixture as in manufacturing usual sodium chromate without any combination with pelletizing. Mr. McCormack applied this method to Cuban ores as early as 1926 but the result showed that the extraction of chromium was quite insufficient (E. Eary: The Aluminum Industry, p. 142). I, the present inventor, have first experimented Omonhon ores by this method. The percentages of extraction were 57.7, 59.0, 63.6 and 87.2% against the amounts of addition of soda ash of 5, 10, 20 and 30%, respectively, at the heating temperature of 700° C. for 30 minutes. These results are not favorable as compared with those of the method of this invention, partly due to the low temperature. After extraction, reheating at a high temperature is necessary to obtain powdered iron ores and briquettes. Thus, this method is unfavorable from the economic point of view.

### (4) SULPHURIC ACID TREATMENT

This method is covered by U. S. Patent No. 2,584,700 on a method of treating iron ores containing nickel and chromium invented by Mr. C. R. Hayward. This patent is owned by Bethlehem Steel Company. This method is also to treat Mayari ores produced in Cuba as summarized in the following. First of all, laterite is treated with sul-

phuric acid. Insoluble chromite and silicic acid are removed. Parts of iron, nickel, aluminum and chromium are then replaced by iron powder thrown in and are precipitated. The remaining iron solution is evaporated, dried and solidified as iron oxide. Sulphur dioxide produced therefrom is utilized for solution. However, the operation in this method is complicated and cannot help being uneconomical, being not a method suited to treatment of large quantities.

An object of this invention is to provide an improved industrial method of extracting chromium from iron ores containing chromium and particularly from laterite.

Another object of this invention is to provide a method of making iron ores containing chromium and particularly laterite raw materials suitable for producing iron.

Further objects of this invention will become clear from the following description.

According to the method of this invention, soda ash and/or lime are added to laterite and the mixture is ground and mixed. The mixture is molded into pellets and is roasted in an oxidizing atmosphere in a furnace to convert chromium contained in the laterite ore into sodium chromate. Then, by immersing the roasted products in water or a solvent, the sodium chromate content is dissolved out and the solid part is separated. Chromium is recovered from the solution. The remaining solid part has very low chromium content and is very suitable as a raw material for producing iron.

Figure 1 of the drawings is a flow sheet showing a mode of working the method of this invention.

Figure 2 shows the percentages of extraction of Cr, Na, Al and SiO<sub>2</sub> when 15% Na<sub>2</sub>CO<sub>3</sub> and various percentages of Ca(OH)<sub>2</sub> were added to laterite and the mixture was treated by the method of this invention.

Figure 3 shows the constitution of pellets obtained by adding 15% Na<sub>2</sub>CO<sub>3</sub> and various percentages of Ca(OH)<sub>2</sub> to laterite as in the case of Figure 2 and by treating the mixture by the method of this invention.

Figure 4 shows the percentages of extraction of Cr and Al when various amounts of Ca(OH)<sub>2</sub> were added to 12.5, 15, 20 and 25% Na<sub>2</sub>CO<sub>3</sub> and the mixtures were treated by the method of this invention.

Figure 5 shows the weight in percentage of Cr remaining in the pellet obtained by treatment under the same condition as in Figure 4.

In the present invention, laterite alone or with the addition of an adequate amount of iron ores or any other raw material for producing iron is first finely ground by means of a grinder. The grinder to be used may be an edge mill or any other known grinder. The size of a ground grain is preferably such as will pass through a 200 mesh screen.

Soda ash or a mixture of soda ash and quick lime in a powdered state in an amount adequate depending on the chromium content is added to the ground iron ores containing chromium and is intimately mixed together. Slaked lime may be used in place of the above quick lime. In mixing them, an adequate amount of water is added for convenience in pelletizing. This water may be fed by adding said soda ash or mixture of soda ash and lime as a solution or suspension. This mixture is then molded into pellets of an adequate size and shape which are preferably of a column 20 to 30 millimeters in diameter and 10 to 20 millimeters long. If the pellet is made a holed pellet by making one or several through-extending holes in the central part thereof, the below mentioned percentage of extraction will be improved, because, in the below mentioned roasting, oxygen will come into contact with the interior of the pellet and, in extracting, the entry of water into the interior will be made easier. When the molded mixture is enclosed in a furnace such as a roasting furnace and is heated at a temperature of 900 to 1200° C. or preferably 1000 to 1100° C. in an oxidizing atmosphere, roasted pellets can be produced. By this heating, the

chromium content in the pellets will be converted to sodium chromate by the following reaction:



In case sodium carbonate Na<sub>2</sub>CO<sub>3</sub> only is used, sodium chromate will be obtained by the following formula:



The sodium chromate thus obtained is very easily soluble in hot water. Therefore, if the roasted pellets while at a high temperature are thrown into and immersed in water which is preferably warm, the greater part of the sodium chromate will be extracted as dissolved. It is preferable to stir the solution in the above immersion. In the above roasting of the pellets the roasted pellets become porous due to the volatilization of water or crystallization of limonite. Therefore, in extracting sodium chromate, water can readily penetrate into the interior of the pellet and sodium chromate can be further dissolved out. Such solvent as, for example, sodium sulphate or calcium carbonate solution may be used instead of the above water. The effects of adding the above soda are as follows:

(1) The iron content is at first limonite but, when heated, becomes hematite. The surface temporarily becomes ferrite due to soda but decomposes and again becomes hematite. A part remains as ferrite but, when made to act with water, becomes hematite and caustic soda. This caustic soda helps the growth of sodium chromate.

(2) Alumina existing as bauxite loses water of crystallization and combines with soda at 550 to 600° C. and leaches out as sodium aluminate, improving the quality of the iron content. The production of alumina as a by-product from ores containing a large amount of alumina and a small amount of silicic acid can be considered.

(3) Silicic acid existing as silica or silica gel combines with soda, becomes sodium silicate and is leached out by water, also serving to improve the quality of the iron content.

The effects of adding lime are as follows:

(1) Lime with the addition of either CaO or Ca(OH)<sub>2</sub> combines with CO<sub>2</sub> obtained by the production of sodium chromate, sodium aluminate or sodium silicate and becomes CaCO<sub>3</sub>, serving to increase the strength of the pellets.

(2) Soda is prevented from acting with alumina or silica and the loss of soda ash is prevented. (In the case of producing alumina as a by-product or of requiring high quality pellets as mentioned above, the amount to be used is limited.)

If the chromium content of the extract obtained by the treatment as mentioned above is concentrated after impurities are removed and is then treated with concentrated sulphuric acid, sodium chromate will become sodium dichromate. It can likewise be made potassium dichromate or chromate by a known method. On the other hand, the pellets from which chromium content has been removed can be used as they are as raw materials for producing iron.

Examples of this invention are shown in the following to help it to be understood. However, this invention is not to be limited to these examples.

#### Example 1

##### PELLETIZING OF IRON ORES CONTAINING CHROMIUM AND ALUMINUM (AN EXPERIMENT BY THE EXTRUSIVE METHOD)

The specimen used in the experiment was Philippine Monhon laterite and its chemical composition was 50.1% Fe, 2.1% Cr, 7.5% Al<sub>2</sub>O<sub>3</sub>, 1.9% SiO<sub>2</sub>, 10.6% combined water and small amounts of Ni, CO, Mn, etc.

This specimen was first ground to grains finer than 200 mesh by means of an edge runner as shown in Fig.

1. Soda ash (sodium carbonate) and slaked lime in a

## 5

state of solution or suspension were added to the above ground specimen and the mixture was well mixed by means of a mixer. Then the mixture was extruded into the shape of a column by means of an Auger type pug mill and was cut into pellets each 20 millimeters in diameter and 10 millimeters long.

These pellets were put into a roasting furnace, were heated for an hour at 1100° C. to 1200° C. in an oxidizing atmosphere, were then thrown while still at a high temperature (about 500° C.) into an extracting tank provided with an agitator and were subjected to extraction for 1 to 2 hours with the water temperature kept at 70 to 80° C. The greater parts of chromium and aluminum were extracted during the first hour and almost all of them were extracted during two hours.  $\text{Al(OH)}_3$  in the extract was first precipitated and roasted to obtain  $\text{Al}_2\text{O}_3$ . The remaining solution was concentrated and was treated with concentrated sulphuric acid to produce sodium dichromate. The percentages of the above extraction were as shown in Fig. 2. As more than 15% Na evaporated in roasting, it could be separately recovered and utilized. As seen in the figure, the percentage of extraction of Cr and Al was the best at 2 to 4% of added  $\text{Ca(OH)}_2$ . The percentage of extraction of  $\text{SiO}_2$  was lower. The percentages by weight of the compositions of the pellet produced by the above-mentioned method were as shown in Fig. 3. They decreased a little with the increase of  $\text{Ca(OH)}_2$  at 60% iron content. With the addition of 3%  $\text{Ca(OH)}_2$ , Fe was 59.0%,  $\text{Na}_2\text{O}$  was 0.4%,  $\text{Al}_2\text{O}_3$  was 2.1% and  $\text{SiO}_2$  was 2.0%. The compressive strength of this pellet was 10 kg. and its specific gravity was 3.45.

The percentages of extraction in case the amount of  $\text{Ca(OH)}_2$  was varied against the amounts of 12.5, 15, 20 and 25%  $\text{Na}_2\text{CO}_3$  are shown in Fig. 4. As seen from said figure, Cr showed the maximum value of 85% at 12.5%  $\text{Na}_2\text{CO}_3$  and more than 90% at both 15 and 20%  $\text{Na}_2\text{CO}_3$ . At 15%, the maximum value of  $\text{Ca(OH)}_2$  was 2 to 4% but, at 20%, it was 6 to 8%. The percentage of extraction at 25%  $\text{Na}_2\text{CO}_3$  was lower than at 20%. It was found that the increase of the amount of extraction of Al in proportion to the amount of addition of  $\text{Na}_2\text{CO}_3$  was more remarkable than that of Cr.

Fig. 5 shows the chromium contents of the pellet produced against the amounts of addition of



shown in Fig. 3. The minima of Cr against 12.5, 15, 20 and 25%  $\text{Na}_2\text{CO}_3$  were 0.42, 0.24, 0.19 and 0.18%, respectively. Especially, with the increase of  $\text{Na}_2\text{CO}_3$ , the strength of the pellet decreased. The compressive strength of 10 kg. of the pellet at 15%  $\text{Na}_2\text{CO}_3$  and 3%  $\text{Ca(OH)}_2$  lowered to that of 7 and 3 kg., respectively at the same percentage of  $\text{Ca(OH)}_2$  but at 20 and 25%

| Examples | Chromium content in the ore | Additives in Percent | Temperatures, °C. | Time (hours) | Chromium Remaining in Pellets in Percent | Amounts of Extraction of Chromium in Percent | Percentage of Extraction of Chromium |
|----------|-----------------------------|----------------------|-------------------|--------------|------------------------------------------|----------------------------------------------|--------------------------------------|
| 5-----   | 2.05                        | 13 soda ash          | 1.000             | 0.5          | 0.40                                     | 1.66                                         | 80.0                                 |
| 6-----   | 2.05                        | do                   | 1.000             | 1.0          | 0.28                                     | 1.77                                         | 86.0                                 |
| 7-----   | 2.05                        | do                   | 1.000             | 2.0          | 0.23                                     | 1.83                                         | 89.2                                 |
| 8-----   | 2.2                         | 10 soda ash, 7 lime  | 1.000             | 0.5          | 0.36                                     | 1.84                                         | 82.7                                 |
| 9-----   | 2.2                         | do                   | 1.000             | 1.0          | 0.26                                     | 1.94                                         | 88.2                                 |
| 10-----  | 2.2                         | do                   | 1.000             | 2.0          | 0.18                                     | 2.03                                         | 92.3                                 |

$\text{Na}_2\text{CO}_3$ . Therefore, the decrease of strength could be compensated by increasing the amount of addition of  $\text{Ca(OH)}_2$ . Generally, the most favorable amount of addition of  $\text{Ca(OH)}_2$  is  $\frac{1}{4}$  to  $\frac{1}{3}$  the amount of addition of  $\text{Na}_2\text{CO}_3$ . However, the absolute values of the amounts of addition of  $\text{Na}_2\text{CO}_3$  and  $\text{Ca(OH)}_2$  vary depending on the composition of the raw material to be used or particularly on the contents of Cr and Al to be extracted and on whether Cr only is to be removed as a by-product or both Cr and Al are to be removed.

## 6

## Example 2

The treatment was the same as in Example 1 with the exception that soda ash alone was added. The result was that the percentages of extraction of Cr at the amounts of addition of 12.5, 15, 20 and 25%  $\text{Na}_2\text{CO}_3$  were 72, 77, 85 and 88.5%, respectively, being less than in the case of simultaneously adding  $\text{Ca(OH)}_2$ .

## Example 3

10 Pellets were made in the same way as in Example 1 except that they were cylindrical pellets each 20 millimeters in diameter and 20 millimeters long with a hole 5 millimeters in diameter made through the center thereof. The amounts of addition in percent of  $\text{Na}_2\text{CO}_3$  and  $\text{Ca(OH)}_2$  and the percentages of extraction of Cr are as shown in the following, those in the case of a pellet without a hole being also shown for information:

| $\text{Na}_2\text{CO}_3$ | $\text{Ca(OH)}_2$ | Percentages of Extraction of Cr |              |
|--------------------------|-------------------|---------------------------------|--------------|
|                          |                   | Cylindrical Pellet              | Holed Pellet |
| Percent                  | Percent           | Percent                         | Percent      |
| 10                       | 12                | 72                              | 90           |
| 12.5                     | 12                | 77                              | 88.5         |
| 15.0                     | 12                | 84                              | 90.0         |

25 As seen in the above, the percentage of extraction of chromium could be increased by 6 to 12% by making a hole in the pellet. Almost the same results were obtained in respect of aluminum.

## Example 4

35 Pellets for producing iron could be made by removing Cr and Al by the same method as in the above from a product from which Ni and Co have been removed by the wet or dry process. Ni and Co were removed by the wet process from ores produced in the Philippines and containing 54.08% Fe, 1.2% Ni, 0.3% Co, 2.92% Cr, 1.92%  $\text{Al}_2\text{O}_3$  and 2.20%  $\text{SiO}_2$ . 20% soda and 4% lime ( $\text{Ca(OH)}_2$ ) were added to the above residues and the mixture was heated for an hour at 1100° C. and was subjected to extraction for two hours. Thus the percentage of extraction of Cr of 85% was obtained.

## Examples 5-10

Laterite ores containing 2.2 and 2.05% chromium, respectively, were ground into grains finer than 200 mesh. 50 Powdered soda ash and quick lime were added to said ground laterite and the mixture was well mixed to be a raw material for pelletizing by a balling mill. The conditions and results were as listed below.

In case the heating temperature was 1100 to 1200° C., the heating time could be further reduced and yet the same results could be obtained.

70 The pellets from which chromium was thus removed contained 57% iron, were good in both strength and reduction rate and could be made raw materials for producing iron as they were.

Now the features of the method of this invention are enumerated as follows:

75 (1) If water is added to laterite in the wet treatment,

it will take a long time for precipitation and drying, such method being uneconomical. The method of this invention wherein the dry treatment is utilized is advantageous.

(2) In this method, the characteristics of laterite are ingeniously utilized and the property which would be very troublesome in the ordinary method proves all the more advantageous.

For example, (i) chromite which is brittle in nature and is apt to be powdered is all the more favorable in completely acting with soda ash. (ii) It is almost impossible to ideally separate limonite adsorbed around chromite. However, in this method wherein the material is finely ground from the first, the above disadvantage has no effect whatsoever. (iii) Iron oxide and alumina have water of crystallization (8.5% at 200 to 250° C.). When the pellet is heated, said water of crystallization will volatilize and the pellet will become porous. This will facilitate the circulation of air, promote the growth of sodium chromate and also facilitate leaching with water, increasing the percentage of removal of chromium.

While this invention has been described in the above chiefly with respect to laterite, it will be easily understood that the same can be applied to any other iron ores containing chromium.

What I claim is:

1. A method of producing pellets containing substantially no chromium, said pellets being suitable as raw material for the production of iron, which method comprises grinding an iron-bearing material comprising chromium and aluminum, adding to the ground material (a) a sufficient quantity of soda ash to convert at least the chromium into a sodium salt thereof and (b) lime in an amount of at least about  $\frac{1}{4}$  the quantity of added soda ash, intimately admixing said materials, adding to the resultant mixture sufficient water to enable the mixture to be molded, molding the aqueous mixture into pellet form, heating the thus-obtained pellets to 900-1200° C. in an oxidizing atmosphere, extracting the thus-treated pellets with an aqueous liquid, whereby at least substantially all the chromium is extracted therefrom.

2. A method according to claim 1, and recovering sodium salt of chromium from the aqueous extract.

3. A method of producing pellets containing substantially no chromium, said pellets being suitable as raw material for the production of iron, which method comprises grinding an iron-bearing material comprising chromium and aluminum, adding to the ground material (a) a sufficient quantity of soda ash to convert at least the chromium and aluminum into sodium salts thereof and (b) lime in an amount of at least about  $\frac{1}{4}$  the quantity of added soda ash, intimately admixing said materials, adding to the resultant mixture sufficient water to enable the mixture to be molded, molding the aqueous mixture into pellet form, heating the thus-obtained pellets to 900-1200° C. in an oxidizing atmosphere, extracting the thus-treated pellets with an aqueous liquid, whereby at least substantially all the chromium and aluminum are extracted therefrom.

4. A method according to claim 1, wherein the heating of the pellets is carried out at 1000 to 1100° C.

5. A method according to claim 1, wherein the iron-bearing material is laterite ore.

6. A method according to claim 1, wherein the pellets are extruded into hollow pellet form.

7. A method according to claim 1, wherein the aqueous liquid is warm water.

8. A method according to claim 1, wherein the molding into pellet form is effected by extrusion.

9. A method according to claim 1, wherein the molding into pellet form is effected in a balling mill.

30 References Cited in the file of this patent

UNITED STATES PATENTS

|           |          |               |
|-----------|----------|---------------|
| 1,832,069 | Wechter  | Nov. 17, 1931 |
| 2,279,033 | Dolbear  | Apr. 7, 1942  |
| 2,381,236 | Udy      | Aug. 7, 1945  |
| 2,381,565 | Udy      | Aug. 7, 1945  |
| 2,402,103 | Udy      | June 11, 1946 |
| 2,430,261 | Udy      | Nov. 4, 1947  |
| 2,592,421 | Heilmann | Apr. 8, 1952  |

FOREIGN PATENTS

|         |               |             |
|---------|---------------|-------------|
| 270,143 | Great Britain | May 5, 1927 |
|---------|---------------|-------------|